

# UNITED STATES PATENT OFFICE.

CHRISTOPHER J. HEIDORF, OF GLENS FALLS, NEW YORK.

## BINDING COMPOSITION FOR WALL-PAPER COLORS.

1,358,151.

Specification of Letters Patent.

Patented Nov. 9, 1920.

No Drawing.

Application filed October 7, 1919. Serial No. 328,971.

To all whom it may concern:

Be it known that I, CHRISTOPHER J. HEIDORF, a citizen of the United States, residing at Glens Falls, in the county of Warren, 5 State of New York, have invented certain new and useful Improvements in Binding Composition for Wall-Paper Colors; and I do hereby declare the following to be a full, clear, and exact description of the invention, such as will enable others skilled in the art to which it appertains to make and use the same.

This invention relates to compositions for use as binders in the printing of wall paper.

15 The composition is intended to be used as a substitute for the ordinary binder varnish and forms a vehicle for the color. In practice, the composition has a sizing effect at the same time that it acts as a vehicle.

20 In the manufacture of my improved composition, I use the ingredients in the proportions as follows:

|                      |                |          |
|----------------------|----------------|----------|
| Cold water           | 3              | gallons. |
| Kerosene oil         | $\frac{1}{2}$  | gallon.  |
| Boiled linseed oil   | 1              | quart.   |
| Soap powder          | $1\frac{1}{2}$ | pounds.  |
| Tapioca flour powder | 2              | pounds.  |

In the assembly of the above named ingredients, the cold water is provided and to it are added the other ingredients in any convenient order and after being thoroughly

mixed, they are boiled together until there is a resultant pasty mass. The mass is then permitted to cool and when cold, it is ready 35 for use.

The composition is employed in place of the usual compound of resin and turpentine as a sizing or binder for binding the color to the paper.

40 What is claimed is:

1. A binding composition for use in the printing of wall paper, consisting of water, kerosene oil, boiled linseed oil, soap powder and tapioca flour.

45 2. A binding composition for use in the printing of wall paper, comprising the following ingredients in the proportions substantially as stated, water 3 gallons, kerosene oil  $\frac{1}{2}$  gallon, boiled linseed oil 1 quart, 50 soap powder  $1\frac{1}{2}$  pounds, and tapioca flour powder 2 pounds.

3. The method of producing a composition for use as a binder in the printing of wall paper, which consists in assembling in a cold 55 state, water, kerosene oil, boiled linseed oil, soap powder and tapioca flour and then boiling the mass until it is pasty.

In testimony whereof, I affix my signature, in the presence of two witnesses.

CHRISTOPHER J. HEIDORF.

Witnesses:

THOMAS H. HEIDORF,  
W. I. LOCKE.